

## UNITED STATES PATENT OFFICE

2,418,879

PYROLYSIS OF HYDROCARBONS TO  
PRODUCE OLEFINESJohn H. Haslam, Louisville, Ky., assignor to The  
Girdler Corporation, Louisville, Ky., a corpora-  
tion of DelawareNo Drawing. Application February 29, 1944,  
Serial No. 524,464

12 Claims. (Cl. 260—680)

**1** This invention relates to the production of olefines by pyrolysis of hydrocarbons by the action of a heated alkaline earth oxide catalyst.

In ordinary practice the hydrocarbon is vaporized, usually mixed with an inert gas such as steam or nitrogen, and then passed over the catalyst at an elevated temperature. Under proper conditions, a portion of the hydrocarbon is converted into the desired olefine, and there is also produced free carbon and a mixture of other undesired decomposition products. The carbon so formed deposits in the reaction chamber and often accumulates to the point where it blocks the chamber and coats the catalyst so as to quickly render it no longer effective for the purpose of olefine production. When this condition is reached, the operation has to be stopped and the catalyst changed or treated in situ by oxidation to remove carbon. This is a costly and time-consuming operation. Furthermore, the production of such carbon and other decomposition product is the result of an undesired reaction and results in a lower yield of the desired olefine.

**2** other decomposition products. The undecomposed cyclohexane could be separated from the butadiene and other decomposition products, and recirculated over the catalyst. Carbon deposited at such a rate that after 2 hours operation the catalyst was coated with carbon, which comprised 0.5% by weight of the catalyst. As the deposition of carbon continues, the butadiene yield decreases, and in a comparatively short time the tubes become plugged with carbon.

In an effort to discover some means for repressing the deposition of carbon on the catalyst, and also in an effort to discover some means of increasing the butadiene yield, a series of tests have been made to determine the effect of preheating the catalyst on these factors, and the results are shown in the following table. In obtaining the data for this table the percentages given are those obtained by a single passing of cyclohexane over the catalyst, calcium oxide, at a temperature of 650° C., and after the catalyst had been preheated to the temperatures and for the times stated.

*Effect of preheating of catalyst*

| Time of Pre-heating, Hrs. | Temper-ature of Pre-heating, °C. | Per cent of Carbon on Catalyst After use for 2.0 Hrs. | Per cent of Cyclohexane decomposed (by weight) | Per cent of Butadiene in Products of Decomposi-tion (by weight) | Per cent of Cyclohexane converted to butadiene (by weight) |
|---------------------------|----------------------------------|-------------------------------------------------------|------------------------------------------------|-----------------------------------------------------------------|------------------------------------------------------------|
| 0                         |                                  | 0.5                                                   | 10.6                                           | 24.5                                                            | 2.60                                                       |
| 22                        | 100                              | 0.6                                                   | 10.4                                           |                                                                 |                                                            |
| 22                        | 200                              | 0.9                                                   | 12.6                                           | 24.5                                                            | 3.10                                                       |
| 22                        | 400                              | 0.5                                                   | 17.8                                           | 17.8                                                            | 3.17                                                       |
| 6                         | 875                              | 0.4                                                   | 7.3                                            | 20.7                                                            | 1.51                                                       |
| 4                         | 1,100                            | 0.0                                                   | 4.0                                            | 18.0                                                            | 0.72                                                       |

Obviously, it is desirable to provide a process in which the yield of the olefine is increased, and also to provide a process in which the deposit of the carbon is decreased.

I have discovered that by certain pretreatment of the alkaline earth oxide catalyst by controlled heating, I can accomplish these desired results.

A procedure following the teachings of the prior art is one in which cyclohexane vapors are mixed with an equal volume of nitrogen and passed over lumps of calcium oxide at 650° C. at 500 space velocity. By "space velocity" is meant the volume of gas under standard conditions of temperature and pressure, introduced per hour per volume of catalyst. As a result, 10% of the cyclohexane was decomposed, 23% of the cyclohexane that was decomposed formed butadiene, and the other 77% formed carbon and

From the data given in this table it will be seen that when the catalyst was preheated to 875° C. to 1100° C., the carbon deposit on the catalyst was almost entirely or entirely eliminated, but the percentage of cyclohexane which was decomposed was decreased, and the percentage of the decomposition product which was the desirable butadiene, was somewhat decreased. It will be noted that by preheating the catalyst to 1100° C. for 4 hours, and then using the catalyst at 650° C. for pyrolysis of cyclohexane, the deposition of carbon on the catalyst was eliminated, but the activity of the catalyst was reduced to such an extent that only 4% of the cyclohexane was decomposed, and of that, only 18% was butadiene. Therefore, the pretreatment at elevated temperatures, and especially in a range above 400° C., had the desirable effect of largely eliminating carbon deposi-

tion but the undesirable effect of reducing the yield of butadiene. The latter is not so important, as the undecomposed cyclohexane may be recycled.

It will also be noted that when the catalyst was preheated at 200° C. for 22 hours, and then used at 650° C. for 2 hours, for the pyrolysis of cyclohexane, the deposition of carbon on the catalyst was increased to 0.9%, but in spite of the increase in carbon deposition, advantageous results were obtained, in that the percentage of cyclohexane decomposed was increased to 12.8%, and the yield of butadiene was increased to 3.10%.

In a preferred embodiment of the present invention the calcium oxide is preheated in a 2-stage heating process, although in carrying out the invention, either stage may be used alone, depending upon the results desired. In the first stage the calcium oxide is heated for at least one hour to a temperature above that at which it is to be used in the pyrolysis reaction, and in the second stage it is held at a temperature below that at which it is used in the pyrolysis reaction for at least four hours. What changes are effected in the calcium oxide in these preheating stages is not known, but tests show that by these preheating steps, less carbon deposit is obtained and higher yields of butadiene are obtained.

One way in which this invention has been carried out is as follows: The catalyst was preheated in two stages, while a gas such as nitrogen, oxygen, or other gas, which was inert so far as action on the catalyst was concerned, was passed over it. The preheating in the first stage was to a temperature of 1100° C. for a period such as 2 hours, and then the temperature was maintained in the second stage at about 200° C. for a longer period, such as 22 hours. The changes effected in the catalyst were of such a character that when the catalyst was used at 650° C. for pyrolysis of cyclohexane, satisfactory results were obtained. In one such test 8.9% of the cyclohexane was converted to decomposition products containing 39.1% of butadiene, and with substantially no deposition of carbon on the catalyst. 39.1% of the 8.9% gave a yield of 3.48%, as against a maximum of 3.17% shown in the table. The higher percentage of butadiene in the decomposition products is obviously more important than a high percentage of cyclohexane decomposed, because the undecomposed cyclohexane is separated from other decomposition products after each pass, and is recycled over the catalyst. Tests indicate that the high initial preheating of the catalyst should be to temperatures above 850° C. but not above 1300° C. As the time of preheating at 850° C. is increased, the operation of the catalyst in use is improved, and as the temperature of preheating is increased above 850° C., shorter preheating times are required. Tests indicate that the later holding at a low temperature should be between 100° C. and 400° C. for more than 4 hours. The best results seem to be by using a temperature between 1000° C. and 1200° C. for 2 to 4 hours in the first stage, and a temperature of about 200° C. for about 20 hours in the second stage.

The above ranges of temperature and time are suggested as suitable operating ranges, though I do not limit myself to these conditions, since the invention is of a broader nature, and either heating stage may be used alone. The treating of a catalyst at high temperatures is important for obtaining certain advantages and the treatment of the catalyst at lower temperatures is important for obtaining other advantages.

Although calcium oxide is the catalyst employed in the tests above referred to, it will be apparent that the same preheating treatment may be applied to advantage with other alkaline earth oxide catalysts used for this type of reaction, and that pyrolysis of other hydrocarbons may be effected to produce other olefines.

Having thus described my invention, what I claim as new and desire to secure by Letters Patent is:

1. The process of securing a decrease of carbon deposit on a catalyst composed essentially of an alkaline earth oxide, and during pyrolysis of a hydrocarbon to form an olefine, which includes preheating the catalyst for more than one hour to a temperature above that at which pyrolysis is to be effected but not substantially above 1300° C., and then passing the hydrocarbon over the catalyst at the pyrolysis temperature and without intermediate cooling below the pyrolysis temperature.
2. The process of producing an olefine by pyrolysis of a hydrocarbon in the presence of a catalyst composed essentially of an alkaline earth oxide, and effecting reduction in the deposit of carbon during said pyrolysis, which includes preheating said catalyst for at least an hour to a temperature above that at which pyrolysis is to be effected and to at least 850° C. but not substantially above 1300° C., and directly thereafter passing the hydrocarbon over said catalyst at the pyrolysis temperature.
3. The process of effecting pyrolysis of cyclohexane to butadiene and reducing carbon deposition during said pyrolysis, which includes preheating a catalyst composed essentially of calcium oxide for at least one hour at a temperature between 850° C. and 1300° C., and directly thereafter passing the cyclohexane over the catalyst at the pyrolysis temperature.
4. The process of increasing the yield of the olefine in the pyrolysis of a hydrocarbon in the presence of a catalyst composed essentially of an alkaline earth oxide, which includes preheating said catalyst for more than four hours at a temperature above 100° C. and below that at which pyrolysis is to be effected, directly thereafter heating the catalyst to the temperature at which the pyrolysis is to be effected and passing the hydrocarbon over the catalyst.
5. The process of producing an olefine by pyrolysis of a hydrocarbon in the presence of a catalyst composed essentially of alkaline earth oxide, and effecting increase in the yield of olefine, which includes preheating said catalyst for a period of at least four hours to a temperature below that at which pyrolysis is to be effected and within the range of about 100° C. to about 400° C., and then passing the hydrocarbon over said catalyst at the pyrolysis temperature and without intermediate cooling of the catalyst below said preheat temperature range.
6. The process of effecting pyrolysis of cyclohexane to butadiene and securing increased yield of butadiene, which includes preheating a catalyst composed essentially of calcium oxide for about twenty hours at a temperature below that at which pyrolysis is to be effected and within the range of about 100° C. to about 400° C., and then passing the cyclohexane over said catalyst at the pyrolysis temperature and without intermediate cooling of the catalyst below said preheat temperature range.
7. The process of producing an olefine by the pyrolysis of a hydrocarbon in the presence of a

catalyst composed essentially of an alkaline earth oxide, which includes preheating said catalyst for a period of at least one hour at a temperature above that at which pyrolysis is to be effected but not substantially above 1300° C., then holding the catalyst for a period of at least four hours at a temperature of at least 100° C. but below that at which pyrolysis is to be effected, and directly thereafter heating the catalyst to a temperature at which pyrolysis is to be effected and passing the hydrocarbon over the catalyst.

8. The process of producing an olefine by pyrolysis of a hydrocarbon which includes preheating a catalyst composed essentially of an alkaline earth oxide at a temperature above 650° C. but not substantially above 1300° C. for at least one hour, then preheating said catalyst at a temperature of at least 100° C. but not substantially above 400° C. for at least four hours, and then passing the hydrocarbon over the catalyst at a pyrolysis temperature of about 650° C. but without intermediate cooling of the catalyst below said last mentioned preheating range.

9. A process which includes preheating a catalyst composed essentially of an alkaline earth oxide, to a temperature between 850° C. and 1300° C. for more than one hour, then holding said catalyst at a temperature between 100° C. and 400° C. for more than four hours, and directly thereafter heating the catalyst to a pyrolysis temperature of over 400° C. and less than 850° C. and passing a hydrocarbon over the catalyst at the pyrolysis temperature to produce an olefine by pyrolysis of the hydrocarbon.

10. The process of producing butadiene, which includes preheating a catalyst composed essentially of an alkaline earth oxide, at a temperature above 650° C. but not substantially above 1300° C. for at least one hour, then heating said catalyst at a temperature of at least 100° C. but below 650° C. for at least four hours, and then passing cyclohexane over the catalyst at a pyrolysis temperature of about 650° C. without intermediate cooling of the catalyst below the tem-

perature range of said second preheating step, to thereby produce the butadiene by pyrolysis of the cyclohexane.

11. The process which includes preheating a catalyst composed essentially of calcium oxide, for at least one hour at a temperature of at least 850° C. but not above 1300° C., then permitting said catalyst to cool to a temperature within the range of 100° C. to 400° C., and holding it in that 10 temperature range for more than four hours, and directly thereafter heating the catalyst to a pyrolysis temperature of over 400° C. and less than 850° C. and passing cyclohexane over the catalyst to produce butadiene by pyrolysis of the cyclohexane.

12. The process of effecting pyrolysis of cyclohexane to butadiene, which consists in heating a catalyst, composed essentially of calcium oxide, to a temperature of about 1100° C. for about two hours, then holding said catalyst at about 200° C. for about twenty hours, and directly thereafter heating the catalyst to a pyrolysis temperature of about 650° C. and passing the cyclohexane thereover.

JOHN H. HASLAM.

#### REFERENCES CITED

The following references are of record in the file of this patent:

#### UNITED STATES PATENTS

| Number    | Name     | Date         |
|-----------|----------|--------------|
| 2,274,988 | Matuszak | Mar. 3, 1942 |
| 2,279,198 | Huppke   | Apr. 7, 1942 |

#### FOREIGN PATENTS

| Number  | Country | Date          |
|---------|---------|---------------|
| 307,945 | British | Mar. 11, 1929 |

#### OTHER REFERENCES

Thorpe, "Dictionary of Applied Chemistry," vol. I, p. 732 (1 pge). Longmans, Green & Co., New York (1921). (Patent Office Library.)